

Feb. 16, 1971

R. G. WEST

3,563,897

FERROMAGNETIC GARNET WITH STRESS INSENSITIVE  
B-H LOOP AND METHOD OF MAKING SAME

Filed April 3, 1968

2 Sheets-Sheet 1



INVENTOR  
RUSSELL G. WEST

BY  
Cushman Shchter Cushman  
ATTORNEYS

Feb. 16, 1971

R. G. WEST

3,563,897

FERROMAGNETIC GARNET WITH STRESS INSENSITIVE  
B-H LOOP AND METHOD OF MAKING SAME

Filed April 3, 1968

2 Sheets-Sheet 2



EFFECT OF MECHANICAL  
COMPRESSIVE STRESS ON  
THE HYSTERESIS LOOP  
OF  $\text{Y}_3\text{Fe}_5\text{O}_{12}$

*Fig. 3.*

EFFECT OF MECHANICAL  
COMPRESSIVE STRESS ON  
THE HYSTERESIS LOOP OF  
 $\text{Y}_{2.925}\text{Ce}_{0.075}\text{Fe}_5\text{O}_{12}$

*Fig. 4.*



EFFECT OF MECHANICAL  
COMPRESSIVE STRESS ON  
THE HYSTERESIS LOOP  
OF  $\text{Y}_{2.85}\text{Ce}_{0.15}\text{Fe}_5\text{O}_{12}$

*Fig. 5.*



INVENTOR  
RUSSELL G. WEST

BY *Cushman, Darby & Cushman*  
ATTORNEYS

## 1

3,563,897

## FERROMAGNETIC GARNET WITH STRESS INSENSITIVE B-H LOOP AND METHOD OF MAKING SAME

Russell G. West, Alexandria, Va. (9% Trans-Tech, Inc., 12 Meem Ave., Gaithersburg, Md. 20760)  
Filed Apr. 3, 1968, Ser. No. 718,536  
Int. Cl. C04b 35/40

U.S. Cl. 252—62.57

11 Claims

## ABSTRACT OF THE DISCLOSURE

Yttrium iron garnet ferrites, wherein the introduction of cerium oxide into the garnet reduces the mechanical pressure stress dependence of remanent magnetization and coercive force, are disclosed.

## BACKGROUND OF THE INVENTION

Ferromagnetic garnet materials have been widely used, especially in microwave devices, since their discovery. It has, however, been noted that the yttrium iron garnet does not adequately satisfy certain design requirements for optimum microwave devices.

Yttrium iron garnet ferrites (hereinafter YIG ferrites), will produce a rotation of a plane of polarization of an incident plane polarized electromagnetic wave when properly disposed in a wave guide and biased by a magnetic field. The direction of the biasing magnetic field determines the manner in which the high frequency energy is affected. This property of ferrite materials has resulted in the development of nonreciprocal devices which utilize this rotation, commonly known as the Faraday rotation.

The prior art has substituted certain other ions in the YIG structure for certain magnetic effects. For instance, the Geller U.S. Pat. No. 3,006,855 discloses the use of garnet compounds such as calcium-tin garnets used in solution with YIG ferrites or other rare earth iron garnets, to produce ferrites with magnetic moments substantially higher than that of pure rare earth iron garnet. The Harrison et al. U.S. Pat. No. 3,132,105 discloses the incorporation of gadolinium in YIG ferrites to produce a relatively low saturation magnetization value, which remains substantially constant over an extended range of temperature values. A similar disclosure is found in the Zneimer et al. Pat. No. 3,125,534. The Geller Pat. No. 3,006,854 discloses incorporation of zirconium or hafnium ions into YIG ferrite structures.

One of the problems encountered by the user of YIG ferrites in microwave applications relates to stress-induced changes of magnetization. Mechanical stresses induce a variation of the remanent magnetization of YIG ferrites. That is, tensile or compressive stresses will alter the remanent magnetization of YIG ferrites, as well as altering the coercive force and the shape of the B-H hysteresis loop, of the ferrites. This effect is especially noticeable when a ferromagnetic toroid is utilized in microwave digital phase shifters. The toroid is rigidly located in a wave guide, and any change in tensile or compressive stresses, such as, for instance, those caused by temperature changes, will result in an alteration of the differential phase, since the phase shift is directly related to the remanence magnetization magnitude. This magnetization dependency upon stress is described by Stern and Temme, IEEE Trans. MTT, vol. 3, p. 873 (1965).

Comstock and Raymond, "Journal of Applied Physics," vol. 38, No. 9, p. 3,737 (August 1967) attempted to determine theoretical magnetostriction data for ytterbium and cerium iron garnets. The authors measured the temperature dependence of various constants of  $Yb^{3+}$  in YIG and of  $Ce^{3+}$  in YIG. The cerium iron garnet values

## 2

were determined by testing ferrites made by doping single crystals of YIG with cerium ions. These measurements allowed the authors to make theoretical predictions of the temperature dependence of certain magnetostriction constants of pure ytterbium iron garnet and pure cerium iron garnets (which cannot be grown per se).

Dillon and Neilsen "Physical Review," vol. 120, No. 1, pp. 105-113 (Oct. 1, 1960) performed resonance experiments on single crystals of YIG doped in a melt with rare earth ions, including  $Ce^{+++}$ . The authors found no significant effects in the cerium doping.

Blasse and Bril, "Applied Physics Letters," vol. II, No. 2, pp. 53-55 (July 15, 1967) added  $Ce_2O_3$  to  $Y_2O_3$  and hydrated alumina to produce  $Y_3Al_5O_{12}$ -Ce garnets. Chemical analysis excluded other oxidation states of cerium than  $Ce^{3+}$ . The garnet showed a bright yellow emission under excitation with cathode rays as well as with blue radiation, suggesting the use thereof for phosphors for flying-spot cathode-ray tubes for color television ( $Y_3Al_5O_{12}$  is known to be non-magnetic).

## SUMMARY OF THE INVENTION

Yttrium iron garnet ferrites with stress insensitive B-H hysteresis loops are produced by incorporating cerium oxide into the oxide mixture prior to the firing of oxides to produce the garnet ferromagnetic material. Generally, from about 0.5 to about 7.5 mole percent of the cerium oxide, based on the moles of total oxide, will be utilized. The remanent magnetization of the resultant ferrites is relatively insensitive to tensile and compressive stresses, and the ferrites are particularly suitable for use in microwave differential phase shift devices.

## DESCRIPTION OF THE INVENTION

The introduction of oxides of cerium into yttrium iron garnet has an appreciable effect in controlling the stress dependence of the remanent magnetization of the ferrite. In addition, the coercive force of the YIG ferrite can be made stress-insensitive for quite large variations in mechanical stress. The microwave properties of the resultant ferrite are not appreciably deteriorated. To date, single crystals of YIG have been only of academic interest as toroids in microwave digital applications. It will therefore be appreciated that the present invention is concerned only with polycrystalline garnet structures, wherein the structure is of reduced stress dependency of B-H loops.

The microwave garnets of the present invention can be produced by conventional processes. In one process, the carefully weighed raw materials are first wet mixed with water, in a steel ball mill which preferably has a rubber or plastic lining. Other blending apparatus, such as high-speed blenders, colloid mills and attritors may be used. The resultant homogeneous mixture is then oven dried or spray dried. In this drying operation, water should be removed quite rapidly in order to minimize preferential settling of denser or larger particles. If desired, the mixture may be pressure filtered before drying to expedite water removal.

The dried material may then be presintered, or calcined, by heat treating at a temperature somewhat lower than the final firing temperature. This presintering step generally helps control shrinkage in the final stage and improves homogeneity. All or any portion of the material may be presintered as desired, as known to the art. After the presintering step, the material is comminuted to a particle size that is ceramicallly workable, preferably about two microns or less in size.

Several means of forming the comminuted particles into the desired shapes may be utilized, including die pressing, extruding and hydrostatic or isostatic pressing.

Organic additives may be introduced at this point to serve as a binder and particle lubricant, as desired.

The ferromagnetic ferrites are produced by a solid state reaction at temperatures of 1100 to 1500° C. If an organic additive is used, the formed shapes must be heated gradually during the low temperature range in the firing cycle in order to slowly volatize the organic additive. (Rapid evolution of vapors may crack the formed shapes.)

Hot pressing, which involves the simultaneous pressing and firing of the ferrite, may be used to advantage in many instances. The concurrent application of heat and pressure generally produces good control of density and crystal grain size.

It is known that ferrite materials are generally susceptible to changes in oxygen content during firing. It is therefore preferred to control the chemical valence of the compounds by precise firing schedules and controlled atmospheres during the heat treatment, as known to the art.

The YIG ferrites can be produced by the methods disclosed in U.S. Pats. Nos. 3,131,082, 3,062,746 or 3,051,656, the disclosures of which are hereby incorporated by reference.

Any one or several of the rare earths of atomic number 62-71 may be substituted for a portion of the yttrium in the ferrite of the present invention. Of these, gadolinium is the preferred material. Also, the iron may be replaced in part by aluminum, gallium, or indium, of which aluminum is the most preferred. Such replacements or substitutions will be by way of additions of the respective oxides (or precursors) in lieu of the replaced or substituted oxide. As used herein, unless otherwise specified, the term yttrium iron garnet is to be construed to mean yttrium with and without the presence of up to about 40 weight percent of the garnet of oxides of the rare earths of atomic number 62-71 and with and without the additional presence of oxides of aluminum, gallium or indium as partial substitution (up to 11 weight percent of the garnet) for the iron.

The garnet structure of the present invention will therefore be represented by the following composition:



wherein Z is yttrium alone or mixed with minor amounts (up to about 40 weight percent of the garnet) of oxides (or precursors) of rare earths of atomic numbers 62 to 71 inclusive, A is Fe or Fe mixed with up to about 11 weight percent of the garnet of oxides (or precursors) of Al, Ga or In, and x is a positive number of 0.02 to 0.30. Preferably, Z is pure yttrium or yttrium with up to about 38.5% by weight of the garnet of gadolinium oxide. A is preferably pure Fe or Fe mixed with up to about 10.5% by weight of the garnet of  $Al_2O_3$ . x is preferably 0.05 to 0.15 and most preferably about 0.08. It is to be emphasized that the above formula does not necessarily represent a given compound, but is only indicative of the elements in the garnet composition.

The cerium preferably is added as  $CeO_2$  or a precursor thereof, such as a carbonate, acetate, oxalate, hydroxide and the like, or mixtures thereof. For instance, heating dry cerous carbonate at about 570° C. produces ceric oxide. Kirk-Othmer, "Encyclopedia of Chemical Technology" 2nd Edition, vol. 4 pp. 840-852, the disclosure of which is hereby incorporated by reference, sets forth properties of a number of cerium compounds.

$CeO_2$  is of quite high melting point (2600° C.) which is well above the garnet firing temperatures. The oxidation state of the cerium in the garnet structure is not known. It is possible that the  $Ce^{4+}$  converts, at least in part, to  $Ce^{3+}$  at the sintering temperatures. However, it is to be emphasized that the nature of such a conversion, if any, is not known at this time. The experimental results, as set forth in the working examples below, suggest that the mechanical pressure stress dependency of the remanent magnetization and the coercive force of

YIG garnet ferrites could be reduced by the addition of  $Ce_2O_3$ , or a precursor of  $Ce_2O_3$ , into the oxide starting material mixture. However, the "Handbook of Chemistry and Physics," Chemical Rubber Publishing Co., 36th Edition, indicates that cerous oxide ( $Ce_2O_3$ ) ignites at about 200° C., suggesting that an inert atmosphere would be required. It will therefore be appreciated that the preferred embodiment of the present invention utilizes cerium oxide ( $CeO_2$ ), or precursors thereof.

Regardless of the mechanism by which the cerium oxide is incorporated into the ferrite material, the presence of minor amounts of oxides of cerium render the B-H hysteresis loop stress insensitive, or relatively stress insensitive, which results in reducing the stress dependence of the remanent magnetization (remanent induction) and coercive forces, as well as illustrating a squarer B-H hysteresis loop under stress. The addition of cerium oxide also improves the high power handling characteristics of the garnet.

20 The preferred ferrites of the present invention can be represented by the following atomic composition:



wherein  $y$  is 0 to about 2.0,  $x$  is 0.02 to 0.30, preferably 0.05 to 0.15, and most preferably 0.08, and  $n$  is 0 to about 1.5.

The microwave properties of cerium-containing YIG ferrites are not appreciably deteriorated. The 9.4 GHz. dielectric loss tangent generally remains below about 30 0.0001. The saturation magnetization appears to be relatively insensitive to cerium oxide in the YIG ferrite. The spin wave line width increases rapidly, and the ferromagnetic resonance line width increases moderately, with increasing levels of cerium oxide.

35 The present invention will be more clearly understood from the accompanying drawings, wherein

FIG. 1 is a diagram illustrating the effect of compressive stress upon the remanent induction (remanent magnetization) of YIG ferrites;

40 FIG. 2 is a diagram illustrating the effect of compressive stress upon the coercive force of YIG ferrites;

FIG. 3 is a B-H hysteresis loop for pure unmodified YIG;

45 FIG. 4 is a B-H hysteresis loop for modified YIG, wherein  $x=0.075$ ; and

FIG. 5 is a B-H hysteresis loop for modified YIG wherein  $x=0.15$ .

The methods used to determine the values shown in FIGS. 1 and 2 are described in the Trans-Tech, Inc. advertisement entitled "Test for Hysteresis Loop Properties" appearing in Microwave, Hayden Microwave Corp., New York, N.Y., vol. 5, No. 9, p. 39 (Sept. 1966).

50 A controlled mechanical compressive force was applied into the major axis of the toroid under test. The cerium containing garnets were produced according to the examples of this application (the pure YIG garnet was produced in the same manner as Example 3, with the exception that no  $CeO_2$  was utilized in the mixture, with compensating addition of  $Y_2O_3$ ). All ferrites tested were of the same identical size and shape. 1.86 mole percent  $CeO_2$  represents the situation wherein  $x$  in Formula 1 is 0.075 and 3.68 mole percent  $CeO_2$  represents the situation wherein  $x$  in Formula 1 is 0.15. It will be readily seen that the composition containing 1.68 mole percent  $CeO_2$  is relatively stress insensitive between 0 and 3000 p.s.i. compressive stress, especially when compared to the pure YIG ferrite material.

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8

## 5

A comparison of FIGS. 3, 4 and 5 will show the remarkable improvement in the reduction of stress sensitivity of yttrium iron garnets accomplished by the present invention. The B-H loops of FIGS. 4 and 5 are much squarer under stress and less stress sensitive than the B-H loop of FIG. 3. The compressive stress value of 3000 p.s.i. was arbitrarily chosen for the above tests. The reduction in stress sensitivity obtained by the cerium-containing garnets of the present invention will be noted for much lower and much higher pressures. For instance, the slopes of the curves of FIGS. 1 and 2 indicate that pure YIG ferrite, unlike the compositions of the present invention, is quite stress sensitive at low pressures.

Generally, amounts of cerium oxide in the YIG ferrite corresponding to values of  $x$  in Formula 1 of less than 0.02 will not have an appreciable effect upon the ferromagnetic properties of the resultant garnet. Amounts of cerium oxide greater than that represented by the value of 0.30 for  $x$  in Formula 1 will result in a garnet which is of increasing stress dependency in remanent induction and coercive force, as compared to cerium oxide levels within the ranges herein.

The invention will be understood more readily by reference to the following examples; however, these examples are intended to illustrate the invention and are not to be construed to limit the scope of the invention.

## EXAMPLES OF THE INVENTION

## Example 1

(Preparation of modified YIG garnet of the composition  $Y_{2.925}Ce_{0.075}Fe_5O_{12.}$ )

The following materials were mixed together:

|                                              | Grams  |
|----------------------------------------------|--------|
| $Y_2O_3$ (1.50 micron average particle size) | 44.487 |
| $CeO_2$ (1.65 micron average particle size)  | 1.739  |
| $Fe_2O_3$ (0.5 micron average particle size) | 53.774 |

(All particle sizes were measured on a Fisher Sub-Sieve Sizer.)

The oxides were blended together in a "Waring Blender" with 150 ml. of distilled water for 15 minutes. The resultant slurry was placed in a covered steel pan and heated at 200° C. for about 20 minutes to evaporate the water. The dried cake was then calcined in air at 1250° C. for 8 hours. The calcined powder was placed in a 500 ml. polyethylene jar containing a 1/3 volume charge of 3/8 in. stainless steel balls in 120 ml. of distilled water and milled for 10 hours, at which time the average particle size was less than 2 microns. The resultant milled slurry was dried in a covered steel pan at 200° C. for about 20 minutes. The dried powder was granulated by forcing it through a No. 20 sieve, and then was isostatically pressed into compacts at a pressure of 6000 p.s.i.g. The compacts used in all of the examples were toroids with rectangular outer dimensions of 1 1/2" x 1" x 3/4". A centrally located rectangular hole 1" x 1/8" passed through the compact, opening on the 1 1/2" x 1" sides. The compacts were sintered in oxygen (air) at a temperature of 1480° C. for 10 hours. The sintered ferrites were machined to outer dimensions of 1 1/16" x 3/8" x 3/8". The centrally located hole was not machined, but a volume shrinkage of about 17% was noted. The compressive stresses were applied to the 3/8" x 3/8" sides of the toroid in all B-H load determinations.

The garnet had the atomic composition:



and had the following properties:

|                                         |        |
|-----------------------------------------|--------|
| $4\pi M_s$ (gauss)                      | 1750   |
| $\epsilon'$                             | 14.4   |
| $\tan \delta$ , dielectric loss tangent | 0.0001 |
| $\Delta H$ (oersteds)                   | 130    |
| g-Effective                             | 2.00   |
| $\Delta H_K$ (oersteds)                 | 5.2    |

## 6

The B-H hysteresis loop for the garnet is shown in FIG. 4 of the accompanying drawings.

## Example 2

(Preparation of modified YIG garnet of the composition  $Y_{2.92}Ce_{0.08}Fe_5O_{12.}$ )

The following materials were mixed together:

|                                              | Grams  |
|----------------------------------------------|--------|
| $Y_2O_3$ (1.50 micron average particle size) | 44.393 |
| $CeO_2$ (1.65 micron average particle size)  | 1.854  |
| $Fe_2O_3$ (0.5 micron average particle size) | 53.753 |

The garnet of this example was prepared using the same procedure as described in Example 1.

The resultant garnet structure corresponded to the following atomic composition:  $Y_{2.92}Ce_{0.08}Fe_5O_{12.}$

The garnet had the following intrinsic electrical and magnetic properties:

|                                         |        |
|-----------------------------------------|--------|
| $\tan \delta$ , dielectric loss tangent | 0.0001 |
| $\epsilon'$                             | 14.7   |
| $\Delta H$ (oersteds)                   | 99     |
| $\Delta H_K$ (oersteds)                 | 5.8    |
| g-Effective                             | 1.99   |
| $4\pi M_s$ (gauss)                      | 1600   |

The B-H hysteresis loop of the garnet produced by this example was very similar to that shown in FIG. 4.

## Example 3

(Preparation of modified YIG garnet of the composition  $Y_{2.85}Ce_{0.15}Fe_5O_{12.}$ )

The following oxides were mixed together:

|                                              | Grams  |
|----------------------------------------------|--------|
| $Y_2O_3$ (1.5 micron average particle size)  | 43.088 |
| $CeO_2$ (1.65 micron average particle size)  | 3.457  |
| $Fe_2O_3$ (0.5 micron average particle size) | 53.455 |

The garnet of this example was prepared using the procedure of Example 1, and the garnet had the atomic composition  $Y_{2.85}Ce_{0.15}Fe_5O_{12.}$

The garnet had the following properties:

|                                         |        |
|-----------------------------------------|--------|
| $4\pi M_s$ (gauss)                      | 1760   |
| $\epsilon'$                             | 14.2   |
| $\tan \delta$ , dielectric loss tangent | 0.0001 |
| $\Delta H$ (oersteds)                   | 190    |
| g-Effective                             | 2.03   |
| $\Delta H_K$ (oersteds)                 | 8.6    |

The B-H hysteresis loop for this garnet is shown in FIG. 5 of the accompanying drawings.

## Example 4

(Preparation of modified YIG garnet of the composition  $Y_{2.7}Ce_{0.3}Fe_5O_{12.}$ )

The following oxides were used as starting materials:

|                                              | Grams  |
|----------------------------------------------|--------|
| $Y_2O_3$ (1.5 micron average particle size)  | 40.341 |
| $CeO_2$ (1.65 micron average particle size)  | 6.833  |
| $Fe_2O_3$ (0.5 micron average particle size) | 52.827 |

This example used the procedure of Example I. The garnet had the following electric and magnetic properties:

|                                         |        |
|-----------------------------------------|--------|
| $4\pi M_s$                              | 1780   |
| $\epsilon'$                             | 14.9   |
| $\tan \delta$ , dielectric loss tangent | 0.0001 |
| $\Delta H$ (oersteds)                   | 150    |
| g-Effective                             | 2.02   |
| $\Delta H_K$ (oersteds)                 | 16.6   |
| $T_c$ (° C.)                            | 268    |

While the coercive force of this garnet was of reduced compressive stress sensitivity, the remanent magnetization was much more sensitive to compressive stress than the garnet of Example 3. This suggests that this composition is about the upper limit of  $CeO_2$  addition for the most stress-insensitive B-H loop garnets.

The resultant garnet corresponded to the following atomic composition:



Example 5

(Preparation of modified YIG garnet of the composition  $Y_{2.98}Ce_{0.02}Fe_5O_{12}$ )

A modified YIG garnet was produced utilizing the following raw materials:

|                                              | Grams  |
|----------------------------------------------|--------|
| $Y_2O_3$ (1.50 micron average particle size) | 45.523 |
| $CeO_2$ (1.65 micron average particle size)  | 0.466  |
| $Fe_2O_3$ (0.5 micron average particle size) | 54.011 |

The garnet of this example was prepared using the same procedure as described in Example 1. The resultant garnet had the following atomic composition:



The garnet produced by this example had a B-H loop which was squarer under stress and less sensitive to compressive stresses than the same garnet (of FIG. 3) without the cerium oxide present. The improvement in stress insensitivity was marginal, suggesting that this example may be taken as the general lower working limit of cerium oxide content.

Example 6

(This example relates to a cerium and gadolinium modified YIG garnet of the composition



The oxides used were:

|                                              | Grams  |
|----------------------------------------------|--------|
| $Y_2O_3$ (1.5 micron average particle size)  | 14.608 |
| $CeO_2$ (1.65 micron average particle size)  | 1.591  |
| $Gd_2O_3$ (0.6 micron average particle size) | 37.684 |
| $Fe_2O_3$ (0.5 micron average particle size) | 46.117 |

The garnet was produced using the procedure of Example 1.

The resultant garnet structure corresponded to the following atomic composition:  $Y_{1.12}Ce_{0.08}Gd_{1.8}Fe_5O_{12}$ .

The garnet produced by this example had a B-H loop which was squarer under stress and less sensitive to compressive stresses than the same garnet without the cerium oxide present (compensated by the stoichiometric addition of  $Y_2O_3$ , of course).

Example 7

(This example relates to a cerium and aluminum modified YIG garnet of the composition



The oxides used were:

|                                               | Grams  |
|-----------------------------------------------|--------|
| $Y_2O_3$ (1.5 micron average particle size)   | 49.949 |
| $CeO_2$ (1.65 micron average particle size)   | 1.961  |
| $Fe_2O_3$ (0.5 micron average particle size)  | 40.930 |
| $Al_2O_3$ (1.35 micron average particle size) | 10.160 |

The same process was used as was used in Example 1, except that the compact was sintered in oxygen (air) at a temperature of 1530° C. for 10 hours.

The resultant garnet structure corresponded to the following atomic composition:  $Y_{2.92}Ce_{0.08}Fe_{3.6}Al_{1.4}O_{12}$ .

The garnet produced by this example had a B-H loop which was squarer under stress and less sensitive to compressive stresses than the same garnet without the cerium oxide present (compensated by the stoichiometric addition of  $Y_2O_3$ , of course).

Example 8

(This example relates to the preparation of a cerium, gadolinium and aluminum modified YIG garnet of the composition  $Y_{2.52}Ce_{0.08}Gd_{0.4}Fe_{4.6}Al_{0.4}O_{12}$ )

The oxides used were:

|                                               | Grams  |
|-----------------------------------------------|--------|
| $Y_2O_3$ (1.5 micron average particle size)   | 37.515 |
| $CeO_2$ (1.65 micron average particle size)   | 1.815  |
| $Gd_2O_3$ (0.6 micron average particle size)  | 9.558  |
| $Fe_2O_3$ (0.5 micron average particle size)  | 48.424 |
| $Al_2O_3$ (1.35 micron average particle size) | 2.688  |

The garnet was produced by the procedure of Example 1, except that the compact was sintered in oxygen (air) at a temperature of 1495° C. for 10 hours.

The resultant garnet structure corresponded to the following atomic composition:



The garnet produced by this example had a B-H loop which was squarer under stress and less sensitive to compressive stresses than the same garnet without the cerium oxide present (compensated by the stoichiometric addition of  $Y_2O_3$ , of course).

Obviously many modifications and variations of the present invention are possible in the light of the above teachings. It is, therefore, to be understood that within the scope of the appended claims, the invention may be practiced otherwise than as specifically described.

What is claimed is:

1. Polycrystalline yttrium iron garnet structure of reduced mechanical stress dependency of remanent magnetization and coercive forces consisting essentially of a modified yttrium iron garnet represented by the atomic composition:



wherein Z is selected from the group consisting of yttrium and mixtures thereof with at least one rare earth of atomic numbers 62-71 inclusive the amount of rare earth, calculated as oxide being up to about 40% by weight of the garnet A is selected from the group consisting of iron and mixtures thereof with at least one member selected

from the group consisting of aluminum, gallium and indium, the amount of aluminum, gallium and indium, calculated as oxide being up to about 11% by weight of the garnet, and x is about 0.02 to about 0.30.

2. A composition as claimed in claim 1 wherein x is 0.05 to 0.15.

3. A composition as claimed in claim 1 wherein x is about 0.08.

4. The composition of claim 1 wherein said modified yttrium iron garnet is represented by the atomic composition:



wherein v is 0 to about 2.0, x is about 0.02 to about 0.30, and n is 0 to about 1.5.

5. A composition as claimed in claim 4 wherein v and n are both 0.

6. A composition as claimed in claim 5 wherein x is 0.05 to 0.15.

7. A composition as claimed in claim 5 wherein x is about 0.08.

8. A composition as claimed in claim 1 wherein said rare earth is gadolinium present in an amount, calculated as oxide of up to about 38.5% by weight of the garnet.

9. A composition as claimed in claim 1 wherein A is iron with up to 10.5% by weight of the garnet of aluminum, calculated as oxide.

10. In a process for producing polycrystalline yttrium iron garnet ferrites of the  $Z_3A_5O_{12}$  type wherein Z is selected from the group consisting of yttrium and mixtures thereof with at least one rare earth of atomic numbers 62-71 inclusive, the amount of rare earth, calculated as oxide being up to about 40% by weight of the garnet, and A is selected from the group consisting of iron and mixtures thereof with at least one member selected from

the group consisting of aluminum, gallium and indium,

the amount of aluminum, gallium and indium, calculated as oxide being up to about 11% by weight of the garnet, said process comprising the steps of mixing and blending of raw materials of said yttrium iron garnet ferrites together in the form of oxides or oxide precursors, forming the blended material into formed shapes, and thereafter sintering said formed shapes at temperatures of up to about 1500° C. to obtain ferromagnetic garnets, the improvement comprising adding cerium as an oxide or precursor thereof, as a substitute for a portion of the yttrium, in an amount of from 0.5 to 7.5 mole percent, calculated as oxide, to said raw materials, based on the total moles of raw materials.

11. The process as claimed in claim 10 wherein about 1.86 mole percent of cerium oxide, based on the total number of moles of said raw materials, are added.

## References Cited

## UNITED STATES PATENTS

3,085,980 4/1963 Gorter et al. 252—62.57

## OTHER REFERENCES

Comstock et al.: "Journal of Applied Physics," vol. 39, No. 2, February 1968.

Nilsen et al.: "Journal of Applied Physics," vol. 38, No. 3, March 1967.

TOBIAS E. LEVOW, Primary Examiner

J. COOPER, Assistant Examiner

U.S. CL. X.R.

252—62.58